

E. A. WIDMANN,  
TALKING MACHINE RECORD,  
APPLICATION FILED MAR. 26, 1920.

1,370,719.

Patented Mar. 8, 1921.

Fig.1.



Fig.2.



Inventor

Eugene A. Widmann  
By his Attorney  
Frank L. Ives

# UNITED STATES PATENT OFFICE.

EUGENE A. WIDMANN, OF BROOKLYN, NEW YORK.

## TALKING-MACHINE RECORD.

1,370,719.

Specification of Letters Patent.

Patented Mar. 8, 1921.

Application filed March 26, 1920. Serial No. 369,027.

To all whom it may concern:

Be it known that I, EUGENE A. WIDMANN, a citizen of the United States, and a resident in the borough of Brooklyn, county of 5 Kings, city and State of New York, whose post-office address is No. 10 Grand avenue, Brooklyn, New York, have invented certain new and useful Improvements in Talking-Machine Records, of which the following is a full, clear, and exact description.

My invention relates to various new and useful improvements in talking machine records and my object is to produce a record of superior quality and of low cost.

Experience has shown that shellac is the material *par excellence* for use as a binder in the make-up of compositions for talking machine records, or, at least, for the wearing surface of the same. Such compositions employing shellac as the binding ingredient thereof possess extremely valuable qualities for the purpose. They take a very sharp, clean impression from the matrix so that the record surface is smooth and free 20 from scratch; they possess a very great degree of durability under the wearing action of the stylus which tracks the same; and they are permanent, practically non-hygroscopic and unaffected by changes in temperature encountered under conditions of ordinary use. Furthermore, they do not require a lengthy heat treatment or cooling as is necessary, for instance, when phenolic condensation products are employed. Because 25 of the presence of shellac in these compositions, lending to them the desirable qualities above referred to, they are known in the patent literature of the art as shellac-like material. These compositions differ very 30 largely in their make-up, the shellac being admixed with various fibers and fibrous or amorphous fillers, but they are all characterized by the presence therein of shellac in sufficient quantity to give to the composition 35 the desired physical properties.

The enormous demand for shellac, largely coming from the talking machine art, has made it a very expensive material for use in compositions for talking machine records, 40 and many attempts have been made, therefore, to reduce the amount of shellac used and to confine the shellac-like composition to the record surface or surfaces. Thus attempts have been made to produce composite records with one or more shellac-like 45 record surfaces, and with a non-thermo-

plastic center, such as paper or compositions of wood flour with a suitable binder; but it has been found that when such a record is subjected to heavy pressure necessary to 60 secure the impression of the matrix there is danger of the rough surface of the non-thermo plastic material being reproduced through the shellac-like layer and appearing on the actual record surface as an undesirable roughness producing scratching and other foreign sounds in the reproduction. Moreover, it has been found that with such composite records, although the record 70 surface when initially formed from the matrix is an exact copy thereof, the impression is not permanent and tends to be gradually effaced so that the record becomes undesirably faint.

Other attempts have been made to make 75 composite records by applying a shellac-like layer to a paper sheet and applying the paper sheet so coated to one or both surfaces of a cheap thermo plastic center, the paper being employed to prevent the softer and 80 poorer material from coming through to the surface, and thus reducing the wearing qualities of the record surface. But with these latter records the relatively rough surface of the paper is likely to be formed in 85 the record itself, producing objectionable foreign sounds. Moreover, the records are likely to warp due to uneven expansion and contraction and difficulty has been experienced in preventing undue displacement 90 of the thermo plastic center under the effect of the very great pressures which are imposed in securing the record impressions.

So far as I know, no one has succeeded 95 in making a composite record, with a shellac-like record surface or surfaces, having the desirable practical qualities of a record made wholly of shellac-like material as is the common practice in the art. These composite records as heretofore made have 100 not only been rough but difficulties have been encountered, due to unequal thermo expansion and contraction, resulting in cracks and other physical defects.

Furthermore, the manufacture of such 105 composite records, as heretofore suggested, involves generally an expensive reorganization of factory equipment and change of process, making it difficult and expensive for a concern in actual business to undertake the practical manufacture of the same.

My improved talking machine record is

one in which the record surface itself is just as smooth as when the record is made wholly of shellac-like material. It is just as desirable as a record made wholly 5 of shellac-like material because the surface with which the needle or stylus engages is composed of shellac-like material ordinarily several times thicker than the maximum depth of the record groove. It 10 is just as durable and as no-hygroscopic and, in its other physical properties, as desirable as a record made wholly of shellac-like material, because the additional materials employed are of the same general nature as, though much cheaper than shellac. It is actually superior to a record made 15 wholly of a shellac-like material in the respect that it will resist a higher temperature without change than a record made of shellac-like material (as, for example, if accidentally placed near a radiator) because its melting point is somewhat higher as a 20 whole than shellac.

It possesses the great advantage that it 25 can be manufactured with the same apparatus and by substantially the same process used in the manufacture of records of shellac-like material as now practised in the art.

My invention is based on the discovery 30 made by me that talking machine records, having the desirable properties indicated, can be made by using as a body or foundation to which the shellac-like material is applied, a material practically homogeneous 35 throughout whose melting or softening point is higher than that of shellac. By making a composition record with the central portion of a higher melting or softening point than shellac, the engagement of 40 the matrix during the process of forming the record surface will not unduly deform or displace the central portion, which therefore retains its identity without coming through the surface or weakening by adulteration the film of shellac-like material and 45 the impression will thus be formed solely in the film of shellac-like material.

Materials which I have found admirably adapted for the purpose and which are of 50 a higher melting or softening point than shellac are various gums and resins of the general nature of copal, kauri and dammar and known in the trade as Congo sorts, copal hard sorts, pale East India, Manila 55 sorts, kauri, singapore, dammar, red gum, etc. These materials are all gums or resins whose melting or softening points are higher than shellac and which are hard, uniform and structureless materials. As I shall 60 hereafter point out, in making records it may sometimes be desirable to form the blank of a cheap material with a polished surface to which the film of shellac-like material is applied, and all the materials referred to are capable of taking a very smooth

high polish from a polished mold or matrix. I may use for the center or body portion of my record any one of the foregoing materials or a combination of the same, or any equivalent amorphous, structureless, thermo-plastic material having a higher melting point than shellac. These materials all possess substantially the same coefficients of expansion as shellac or shellac-like materials, so that when the record is completed, 70 as will be explained, its coefficient of expansion is substantially the same throughout and difficulties will not be experienced due to uneven expansion or contraction. At the same time, by properly selecting a suitable combination of these materials in proper proportion, the resulting composition can be made to have the same coefficient of expansion as shellac-like material within very close limits. These gums or 75 resins are capable of being mixed in any desired proportion by simply melting them together.

Instead of using one or more thermo-plastic materials of the general class referred to, with higher melting or softening points than shellac, the center portion of the record may be formed of non-thermo plastic material in a finely divided condition admixed with binders so that the structure as a whole will have a higher melting or softening point than shellac. And such binders themselves may be ones having a higher softening or melting point than shellac or a lower melting or softening point, so long as 90 the composition itself is of such a character that under a temperature which softens the shellac-like film the center of the record would be less affected and more firm and unyielding, so that under the effect of pressure the impression will be formed in the shellac-like film without unduly deforming the central portion of the record. Instead of 95 using gums or resins of the type referred to, either alone or in combination, I may employ for the purpose certain grades of fine asphalt; the melting or softening point of 100 which is higher than shellac.

The important properties which shall be possessed by the material or composition to 115 which the shellac-like material is to be applied are, first, the melting or softening point shall be higher than shellac; second, its coefficient of expansion shall be as near that of shellac as possible; and, third, it 120 shall be structureless and amorphous and preferably in and of itself shall be capable of taking a smooth high polish from a polished mold or matrix. The latter property is especially desirable when the records are 125 made by first forming the central portion or core with a highly polished surface to which the shellac-like material is applied. It is also important that the material to which the shellac-like composition is applied shall 130

not be affected by climatic changes or be subjected to mold or decomposition. If the record impression formed in the shellac-like material is sufficiently deep to produce a deformation in the central material or core, it is also important that this latter material shall possess the property of becoming permanently deformed so that the record impression will be permanent.

10 In making talking machine records according to my invention, I first made an original blank tablet out of the desired material selected, as above explained, and compressed into disks under heat of substantially 15 the diameter but slightly less in thickness than the ultimate record to be secured; or, instead, the material may be pressed into square plates or sheets of the desired thickness from which the disks are finally cut. 20 Preferably, but not necessarily, the disks are pressed and formed between highly polished dies so that their surfaces will be smooth and highly polished. The disks so made are now coated on one or both sides 25 with the shellac-like composition. This is done in any suitable way, as by applying the shellac-like material in a suitable liquid form like paint and allowing it to dry on the surface of the tablet or by applying the shellac- 30 like material in the form of a powder, or by a transfer process by which the shellac-like material in the form of a very thin sheet or film is transferred to one or both surfaces of the disk. The shellac-like material being 35 thus applied to the disk, as explained, the record surface is impressed therein by engaging the shellac-like surface or surfaces between the matrices in a hydraulic or other press in the usual way. During this press- 40 ing operation heat is applied to soften the shellac-like material, whereby a clean-cut smooth impression will be secured without however materially softening, deforming or displacing the main portion of the record, 45 which thus retains its integrity and preserves its general shape and dimensions. This compression of the matrix into the shellac-like material causes the latter to be closely compressed into contact with the 50 body portion of the disk and brings about an effective welding of the shellac-like layer or film thereto, so that practically a homogeneous structure is secured. Thus, at all 55 points the shellac-like film carrying the record surface will be supported intimately by and upon the smooth polished surface of the material of higher melting point, and hence the needle or stylus will be just as rigidly supported by the record as if it were composed of shellac-like material throughout.

60 Instead of making the record, as above described, by first forming a disk of the material of higher melting point and applying a shellac-like film to one or both 65 faces thereof and subsequently impressing

the record grooves in the shellac-like film or films, any other suitable process for producing the improved record may be employed. For example, I may first make the disk or core of the material of higher 70 melting point and then introduce the same between the two matrices of the press, introducing above and below the disk a ball or gob of the shellac-like material of the proper quantity to produce a film of the desired thickness. The matrices being heated and the central disk being also preferably heated at or near the softening point of the shellac-like material the pressure is imparted to the two matrices which thus impose 75 sufficient pressure on the ball or gob of shellac-like material to cause the same to flow and spread evenly over the face of the disk of higher melting point. Thus, the one operation results in the formation of the shellac-like film on the body part of the record and at the same time results in the formation of the record groove therein. Also the shellac-like film will under the effect of heat and pressure be caused to intimately weld to 80 or coalesce with the body part of the record or to form a homogeneous structure.

In order that the invention may be better understood attention is directed to the accompanying drawing forming a part of 90 this specification.

In Figure 1 I illustrate an edge view of a portion of my improved record on an enlarged scale, indicating thereon the center portion composed of "material of higher 100 softening point than shellac" and the two films of "shellac-like material" applied thereto so as to constitute practically a homogeneous structure.

In Fig. 2 I illustrate the bed and plunger of a steam heated hydraulic press, the two matrix faces thereof co-operating with a ball or gob of shellac-like material, as above described, so that when pressure is applied these balls or gobs will be spread 110 out and caused to adhere to the center core and the record impression will be simultaneously formed in the distributed shellac-like material.

Having now described my invention, what 115 I claim as new therein and desire to secure by Letters Patent is as follows:

1. An improved molded sound record, consisting of a practically homogeneous disk formed with a shellac-like record surface 120 and a body portion to which the shellac-like material is welded or coalesced, of a higher melting or softening point than shellac, substantially as set forth.

2. An improved molded sound record, consisting of a practically homogeneous disk formed with a shellac-like record surface and a body part to which the shellac-like material is welded or coalesced, of a structureless, amorphous material of higher melt- 130

ing or softening point than shellac, substantially as set forth.

3. An improved molded sound record, comprising a polished disk of thermo plastic material of higher melting or softening point than shellac and a shellac-like film intimately welded to or coalesced with said disk and carrying a record surface, the record being substantially homogeneous throughout, substantially as set forth.

4. An improved molded sound record, comprising a polished disk of a thermo plas-

tic gum or resin of higher melting or softening point than shellac and a shellac-like film intimately welded to or coalesced with 15 said disk, and carrying a record surface, the record being substantially homogeneous throughout, substantially as set forth.

This specification signed and witnessed this 2nd day of March, 1920.

EUGENE A. WIDMANN

Witnesses:

CATHARINE D. JORDAN,  
M. E. McNINCH.